

## UNITED STATES PATENT OFFICE.

JACQUES COENRAAD HARTOGS, OF ARNHEM, NETHERLANDS.

## SPINNING VISCOSE.

No Drawing.

Application filed June 30, 1924. Serial No. 723,364.

*To all whom it may concern:*

Be it known that I, JACQUES COENRAAD HARTOGS, a subject of the Queen of the Netherlands, residing at Arnhem, Province 5 of Guelderland, Kingdom of the Netherlands, have invented certain new and useful Improvements in Spinning Viscose, of which the following is a specification.

In the art of spinning threads of viscose 10 it is usual to employ spinning baths containing acid by which the viscose is not only coagulated but also decomposed. One of the products of this decomposition is  $H_2S$ . Owing to the rather high temperature of 15 the spinning bath all the  $H_2S$  does not remain in solution, a large portion escaping in gaseous condition. This evolution of gas not only leads to formation of gas-bubbles within the thread, unfavourably affecting its 20 strength and elasticity but also becomes a nuisance because the toxicity of  $H_2S$  makes it necessary to protect the operators and the environments, which is not impossible, but requires complicated and costly processes 25 and apparatus.

It is an object of this invention to eliminate the ill-effects of the sulphureted hydrogen in a manner which does not require complications, considerable expense or a more 30 complicated after-treatment of the spun silk. According to the invention this object is attained by the use of a spinning bath containing one or more ferric salts such as ferric sulphate. The ferric salts may be added to 35 the spinning bath or a ferric compound may be added which forms the desired ferric salt with the acid of the spinning bath.

It is true that  $H_2S$  may be also removed by 40 oxidizing agents but none of these agents conforms with all the requirements. Thus permanganate deposits manganese dioxide which requires an after-treatment with bisulphite or the like. Other oxidizing agents act too strongly and attack the cellulose, 45 some others attack the spinning ducts and accessories and many are impracticable owing to their high price.

Ferric salts, especially ferric sulphate, 50 have none of these drawbacks.

In this case the ferric salt cannot be regarded as an oxidizing agent and is more comparable with  $CuSO_4$  and the like, which combine with  $H_2S$ . These latter, however, 55 form insoluble sulphides, which would have

a detrimental effect. The ferric salt, however, in consequence of the instability of ferric sulphide and the solubility of ferrous sulphide in acids, only yields sulphur and a ferrous salt. It is true that the precipitated sulphur is insoluble, but by its rather low 60 specific gravity its very finely divided state and the fact that it deposits for the major part on the thread and so protects it and because it may be removed entirely afterwards, 65 this sulphur precipitate is an advantage.

It is well-known that finely subdivided sulphur prevents the newly spun threads from adhering to each other and therefore protects the thread from breaking in the 70 twining process.

Ferric salts, such as ferric sulphate as well as the ferrous salts produced may be washed out easily and completely and the oxidizing properties of ferric salts are so extremely weak that there can be no question of attack 75 of the cellulose.

Ferrous salts, especially ferrous sulphate, are easily reoxidized by electrolytic oxidation to ferric salts, which makes it possible to regenerate the spinning bath and to maintain a concentration of ferric salts of any desired degree without being obliged to filter the spinning bath or to renew it or reinforce it more than is the case at present. 80

Ferrous salts, especially ferrous sulphate, have still another valuable property, which they share with zinc sulphate, namely the property of preventing the threads from adhering together and of increasing their lustre. Said property is well-known for 90 zinc-sulphate but is not yet explained.

It is remarkable that by the use of ferric salts the spinning bath is kept absolutely odourless; it seems as if the products which give  $CS_2$  its bad odour such as mercaptans, 95 are made harmless. By the said properties ferric salts are entitled to a quite unique position and cannot be compared with any known means for obtaining the same results.

The concentration of ferric-salts required 100 to remove quickly all  $H_2S$  need be only small; a concentration of 1 per cent is amply sufficient.

What I claim is:

1. In the process of spinning viscose, the 105 step which consists in adding a ferric salt to an acid spinning bath to prevent evolution of sulphureted hydrogen.

2. In the process of spinning viscose, the step which consists in adding ferric sulphate to an acid spinning bath to prevent evolution of sulphureted hydrogen.
3. An acid spinning bath for viscose containing a ferric salt in addition to the usual constituents.

4. An acid spinning bath for viscose containing ferric sulphate in addition to the usual constituents.

In testimony whereof I affix my signature.

JACQUES COENRAAD HARTOGS.